

## UNITED STATES PATENT OFFICE

2,378,699

PROTECTION OF MOLTEN MAGNESIUM AND  
MAGNESIUM-BASE ALLOYSGeorge F. Gunn, Midland, Mich., assignor to The  
Dow Chemical Company, Midland, Mich., a cor-  
poration of MichiganNo Drawing. Application January 16, 1941,  
Serial No. 374,769

10 Claims. (Cl. 22—200)

This invention concerns the protection of exposed surfaces of molten bodies of readily oxidizable metals, such as magnesium and magnesium-base alloys, aluminum, and the like, against attack by the atmosphere.

A number of procedures for protecting the surfaces of molten readily oxidizable metals are known. For example, with magnesium, it is conventional to cover the molten metal with a gaseous blanket of sulfur dioxide, usually by sprinkling sulfur on or near the hot metal. This method is disadvantageous, however, in that frequently violent chemical reaction occurs between the metal and the sulfur, with consequent sputtering, minor flames, and loss. An alternative procedure has been to cover the metal with a protective crust, such as a metal fluoride, and then to strew sulfur on the crust. This method likewise is not overly satisfactory from a practical viewpoint, in that two procedural steps are involved instead of one, and in that the crust, once broken, as by stirring, pouring, or shrinking of the metal, cannot easily be repaired, but must be wholly replaced.

An object of the present invention, then, is to provide an effective means for protecting readily oxidizable metals against atmospheric attack which is extremely simple and yet which avoids the difficulties mentioned.

These objects are attained in the composition of the invention, which consists essentially of a loose mass of a subdivided noncohesive thermostable heat-insulating substance, such as asbestos, which has an apparent specific gravity lower than that of the metal to be protected and is substantially inert chemically thereto, and having admixed therewith a minor proportion of a protective substance, such as sulfur, which when heated in air liberates a gas non-oxidizing toward the metal. In use, the composition is strewed on top of the molten metal in such manner as to cover the exposed surfaces thereof. The asbestos or like material serves as thermal insulation, and the sulfur or other agent evolves a protective gas at a low rate, effectively preventing oxidation of the metal for a long period of time. The protective layer is mobile, and may be parted for stirring or pouring, and then moved back into position after such operation is completed.

As stated, the heat-insulating substance which constitutes the major proportion of the composition should be a loose mass of subdivided material which does not tend to stick together or form a crust on heating, and is preferably in fibrous or granular form. In general, siliceous materials,

especially fibrous siliceous minerals, are the most satisfactory, asbestos, preferably when fluffy, rock wool, glass wool, and exploded mica being commonly used. The gas-forming protective substance in the composition is usually a solid in finely-divided form, powdered sulfur being ordinarily employed, although boric acid or borates, and borofluorides, or mixtures thereof with sulfur are likewise operable. Certain liquids, such as glycerine and other polyhydric alcohols, which liberate protective vapors on heating, may also be used.

In practice the heat-insulating substance and a minor proportion of the protective material, commonly 3 to 10 per cent by weight, are mixed together, either by hand or by machinery, ordinarily just prior to use, and the resulting mass is spread on the metal to be protected, usually as a layer or mat one-half to one and one-half inches thick. If desired, further gas-forming protective material may later be sprinkled upon the insulating layer to replace that consumed during use.

The composition of the invention is particularly convenient for use in preparing castings from metallic magnesium and magnesium-base alloys. In this case, the air in the casting mold is first displaced with a gas non-oxidizing to magnesium, and the molten metal is poured into the mold. All exposed surfaces of the metal in the filled mold are then covered with a layer of the composition, e. g. a mixture of loose fluffy asbestos and sulfur. The sulfur burns slowly to sulfur dioxide which protects the metal against oxidation, while the asbestos prevents too rapid cooling of the top of the casting, thus acting as a "hot top" and minimizing piping. If desired, after cooling, the asbestos layer may be parted, and additional molten magnesium poured into the mold to fill shrinkage losses. When fully solidified, the casting is removed from the mold, any asbestos clinging thereto being brushed off and saved for re-use.

I claim:

1. A composition for protecting surfaces of molten magnesium and magnesium-base alloys against burning which consists essentially of a loose mass of a subdivided noncohesive thermostable heat-insulating siliceous material which has an apparent specific gravity lower than that of the metal and is substantially inert chemically thereto, having admixed therewith a minor proportion of a finely-divided substance which when heated in air liberates a gas non-oxidizing toward the magnesium.

2. A composition according to claim 1 wherein the siliceous material is a fibrous mineral.
3. A composition according to claim 1 wherein the siliceous material is asbestos.
4. A composition according to claim 1 wherein the siliceous material is rock wool.
5. A composition according to claim 1 wherein the siliceous material is exploded mica.
6. A composition for protecting surfaces of molten magnesium and magnesium-base alloys against burning which consists essentially of loose fluffy asbestos having admixed therewith a small proportion of finely-divided sulfur. 10
7. A method of protecting the surfaces of molten bodies of magnesium and magnesium-base alloys which comprises covering the surface with a protective layer consisting essentially of a loose mass of a subdivided noncohesive thermostable heat-insulating siliceous substance having an apparent specific gravity lower than the said metal, and being substantially inert chemically thereto, having admixed therewith a minor proportion of a finely-divided substance which when heated in air liberates a gas non-oxidizing toward the metal. 15
8. A method of protecting the surfaces of molten bodies of magnesium and magnesium-base alloys which comprises covering the surface with 20
- 25 a protective layer consisting essentially of a loose noncohesive mass of a subdivided thermostable heat-insulating siliceous material having an apparent specific gravity lower than that of the metal and being substantially inert chemically thereto, and having admixed therewith a minor proportion of finely-divided sulfur.
9. A method of protecting exposed surfaces of molten magnesium and magnesium-base alloys against oxidation which comprises covering the surface with a protective layer consisting essentially of loose fluffy asbestos having admixed therewith a minor proportion of finely-divided sulfur.
10. In a method of preparing castings from metallic magnesium and magnesium-base alloys, the steps which comprise: displacing the air in a casting mold with a gas non-oxidizing to magnesium, pouring the molten metal into the mold, covering the exposed surfaces of the metal in the filled mold with a protective layer consisting essentially of a mixture of loose fluffy asbestos and a small proportion of finely-divided sulfur, allowing the metal to solidify while thus covered, and removing the casting so formed from the mold. 25

GEORGE F. GUNN.